# EUROPEAN PATENT SPECIFICATION

(11) **EP 2 350 365 B1**
(45) Date of publication and mention of the grant of the patent: **01.05.2019**
(21) Application number: 09821056.0
(22) Date of filing: 09.10.2009
(51) Int. Cl.: D04B 1/14, D03D 15/00, D06P 1/39

(54) **FABRIC INCLUDING POLYURETHANE ELASTIC YARN**
TEXTILES FLÄCHENGEBILDE MIT ELASTOGARN AUS POLYURETHAN
TISSU COMPRENANT UNE FIBRE ÉLASTIQUE DE POLYURÉTHANE

(30) Priority: 13.10.2008 US 104898 P
(43) Date of publication of application: 03.08.2011
(73) Proprietor: Invista Technologies S.à.r.l., 9000 St. Gallen (CH)
(72) Inventor: HIETPAS, Geoffrey, D., Newark, DE 19711 (US); DEWHURST, Robert, Gloucester Abbeydale GL4 4XL (GB)
(74) Representative: Cockerton, Bruce Roger
(86) International application number: PCT/US2009/060143
(87) International publication number: WO 2010/045113

(56) References cited:
- WO-A1-97/49847
- WO-A1-2008/075605
- US-A1- 2002 069 467
- US-A1- 2003 165 677

## Description

### Background of the Invention

### Field of the Invention

Included are fabrics prepared from polyurethane elastic yarn having a cationic dyeable functionality and an acid dyeable yarn. The fabrics can have a uniform color when prepared with separate dye systems.

### Description of Related Art

A fabric that contains elastane (a segmented polyurethane also referred to as spandex) has recognized benefits of comfort, fit, and shape retention. Additionally, it is obvious that consumers value fabrics with a professional looking appearance, which can include having a uniform color. One issue that the fabric industry has failed to address lies in combining the benefits of elastane with uniform color, specifically, the ability to dye the elastane to a shade of similar depth of a companion fiber such as polyamide (nylon). This issue increases with increasing elastane content in the fabric, and in knitted fabrics, including those that have been molded in an extended state. In both cases for knitted fabrics, the inherent stretch in the knitted construction allows for higher fabric stretch and higher yarn movement which exposes the spandex. In the trade the issue of elastane becoming visible in an undesirable manner in a section of fabric that has been stretched is commonly referred to as "grin through".

The inability to dye the elastane a common shade as the companion yarn, especially polyamide, is related to several factors that are common to shade matching any two chemically distinct fibers that dye with the same class of dyes. As an example, acid dyes are used to dye polyamide, silk, and wool, and yet they also are able to stain elastane, thus both fibers dye "together." In addition to differences in affinity and chemical reaction rates between dye molecules and two or more distinct fiber types, depth of shade is widely recognized to also be affected by yarn properties such as decitex, decitex-per-filament in a yarn bundle, and the thermal behavior of the fiber during dye processing conditions.

Previous attempts to combine the benefits of elastane functionality with uniform coloration have attempted to improve the affinity and depth of shade of the elastane with the acid dye types commonly used with polyamide such as U.S. Patent Application Publication No. 2005/0165200 A1 by Selle et al. These efforts are affected by the same difficulties with shade match that resulting from physical and dye uptake differences between the elastane and companion yarns (See for example "Dyeing and Chemical Technology of Textile Fibers" 5th ed. By E.R. Trotman).

Therefore, a need exists for improved stretch fabrics including an elastane yarn and a polyamide yarns and/or proteinaceous yarns that have a more uniform color.

### Summary of the Invention

In some embodiments is an article including a fabric, where the fabric includes a cationic dyeable polyurethane elastic yarn and an acid dyeable yarn. The cationic dyeable yarn may be selected from those disclosed in WO 2008/075605 to OPELONTEX CO., LTD of Japan. The fabric has a uniform color, wherein uniform color means that the color of the fabric as measured by a-color, b-color, and L-value in CIELAB L*a*b* color space is within 10% of the values that are obtained by removing the cationic dyeable polyurethane elastic yarn from the fabric. The fabric includes a cationic dyeable polyurethane elastic yarn dyed by a cationic dye, and an acid dyeable yarn dyed by an acid dye, wherein the acid dyeable yarn is selected from the group consisting of polyamide, proteinaceous, and combinations thereof. The fabric comprises from greater than 0 up to 60% by weight of the cationic dyeable polyurethane elastic yarn.
In another embodiment is a method for preparing a fabric including:
(a) providing a fabric including a cationic dyeable polyurethane elastic yarn and an acid dyeable yarn selected from the group consisting of polyamide, proteinaceous, and combinations thereof,
(b) contacting the fabric with a cationic dye, and
(c) contacting the fabric with an acid dye, wherein the fabric has uniform color, wherein uniform color means that the color of the fabric as measured by a-color, b-color, and L-value in CIELAB L*a*b* color space is within 10% of the values that are obtained by removing the cationic dyeable polyurethane elastic yarn from the fabric;
and wherein the fabric comprises from greater than 0 up to 60% by weight of the cationic dyeable polyurethane elastic yarn.

### Detailed Description of the Invention

Surprisingly, it has been found that one may overcome the deficiencies of a stretch fabric having an elastane yarn and an acid dyeable yarn, by preparing a fabric that includes a unique combination of polyurethane elastic yarn with cationic dye-able functionality as disclosed in WO 2008/075605 and a companion yarn with acid dye functionality.

As used herein, the terms spandex, elastane, and polyurethane elastic yarn are used interchangeably and refer to a segmented polyurethane elastic yarn.

The cationic dyeable polyurethane elastic yarn and the acid dyeable companion yarn can be combined either in the same yarn, or separately combined into the fabric. The fabric can be prepared into any suitable construction including circular knit, warp knit, and woven. After the fabric is prepared, the fabric is separately treated with cationic dyes and acid dyes. Either the cationic dye or the acid dye may be applied first depending on the desired properties of the fabric. The cationic dyeable elastane may be used in a fabric in any suitable amount to provide the desired stretch-recovery property to the fabric. The fabric includes greater than zero and up to about 60% by weight of the cationic dyeable elastane.

Another suitable method for obtaining a uniformly colored fabric is to prepare a knitted or woven fabric with the cationic dyeable elastane and an acid dyeable companion yarn. The fabric is first contacted with an acid dye to achieve the desired shade for the companion yarn using dyes that either do not dye at all or only slightly dye or stain the cationic dyeable elastane. Then the fabric is contacted with a cationic dye to dye the elastane. Dyeing of the elastane yarn of the fabric may occur in a separate step or in the same dye bath where the acid dyeable companion yarn is dyed. When one dye bath is used, the acid dye bath is combined with an alternative dye recipe (such cationic dyes) that have been specifically adjusted for the elastane's unique chemistry and fiber diameter to match the shade of the companion yarn.

Additionally, given that elastane yarns stretch up to 500%, and that shade appearance is dependent on fiber diameter, the elastane color depth can be optimized to match the companion yarn in the relaxed state in a fabric or at a specifically targeted level of extension.

The companion yarn includes an acid dyeable yarn selected from the group consisting of polyamide, proteinaceous, and combinations thereof. Polyamide polymers are well known in the art. They are generally prepared by the condensation polymerization of a dicarboxylic acid and a diamine or the condensation of a monoaminomonocarboxylic acid which is normally derived from its internal lactam. Examples of such polyamides are nylon 6,6 or nylon-6 which are respectively prepared from hexamethylene diamine - adipic acid mixtures and ε-caprotactam. Examples of other fiber-forming polyamides are nylon -6/6,6 copolymers, nylon-11, nylon-12. Examples of proteinaceous fibers include silk, wool, mohair, angora, and alpaca. Combinations of these fibers may be used in the same yarn or single component yarns may be combined into fabric.

Examples of useful acid dyes include Color Index (C.I.) dyes: Acid Yellows 24, 40, 59, 159, 184, 204 and 246, Acid Oranges 142 and 156, Acid Reds 50, 51, 52, 138, 151, 299, 361, 362, Acid Greens 104 and 108, Acid Blues 113, 171, 185, 193, 277 and 324, Acid Violet 90, Acid Brown 298, Acid Blacks 52, 131:1, 132:1, 172, 187 and 194. Examples of useful non-Color Index dyes include: Lanaset Blue 2R, Lanaset Navy R, Lanaset Red G, Lanaset Red 2GA, Lanaset Violet B, Lanaset Brown B, Burconyl Brick Red AF-3b, Burconyl Rubine AF-GR, Burconyl Orange AF-3R, Burconyl Green AF-B, Burconyl Brilliant Blue AF-R, Burconyl Royal Blue AF-R, Burconyl Brilliant Yellow AF-4G, Erionyl Red A-3G, Erionyl Blue RL 200, and Nylanthrene Brilliant Blue 2RFF.

Other useful dyes, including cationic dyes are known in the art and are disclosed in WO 2008/075605.

Color measurements are made on fabrics with a Datacolor Spectraflash Model SF-300 colorimeter (Datacolor International, Lawrenceville, NJ) using a D65/10 degree illuminant. Measurements are reported using the international standard color measurement method promulgated by "Commission Internationale de L'Eclairage" (Paris, France), (International Society for Illumination/Lighting), ("CIE") using standard color coordinates of the CIELAB L*a*b* color space: "L" designates the lightness coordinate; "a" designates the red/green coordinate (+a indicating red and -a indicating green); and "b" designates the yellow/blue coordinate (+b indicating yellow and -b indicating blue). The total color difference between two samples, ΔE, is obtained by taking the difference between the L*, a*, and b* coordinates. The uniform color of the fabrics include where color of the fabric as measured by a-color, b-color, and L-value is within 10% of the values that are obtained by removing the cationic dyeable elastic yarn from the fabric.

### • General Processing Conditions

### • Preparation

- Hose or garment pre-steamed at autoclave temperatures ranging from 85-115C can be used to stabilise garment sizing and to minimise creasing in subsequent wet processing.
- Open Width Fabric Stabilisation, particularly for LYCRA® fibre blends can be achieved in dry heat stenter setting at 160-200C for 60-45 seconds. Depending on fabric quality an anti-oxidant protection may be used in the pad to protect the amine end groups/dye sites of the polyamide during pre-setting (commercial example 2-3%owf Spanscour Spark Tanatex)

### • Scouring

- 1-2g/l non-ionic detergent
- 1-2 g/l Soda at 70-80C for 20 minutes

### • Single Bath 2 stage Method

- Since the solid shade colour effects are based on a combination of anionic and cationic dyes it is important to modify single bath dyeings to facilitate separate exhaustion of the two dye types.
- Cationic dyes strike faster than anionic dyes and should be applied to the dye bath first at the lowest possible temperature, with a cationic levelling agent. Subsequent treatment at 40-70C for 10-30 minutes will achieve substantial exhaustion. Application of the acid dyes, after cooling back to 40C, can then be more safely managed through raise at 1c/ minute to 98c dye 30-60 minutes.

### • Two Bath Method.

Apply the cationic dyes to the spandex as described in the single bath method, cool back and rinse then apply the acid dyes on to the polyamide in a second bath, this will be preferred for very dark shades where there might be a risk of dye precipitation, i.e. cationic dyes that have not exhausted on to the fibre remaining in the dye bath resulting in precipitation of the dyes when the acid dyes are added.

### Dyeing Process Control

- Dyeing by constant pH will ensure the best balance in shade and colour reproducibility although acid donors can be used.
- A constant pH6.5-7.0 will be optimum but sometimes downward adjustment to pH4.5-5.5 will be required to achieve dye exhaustion. It is important to set the pH before the addition of the cationic dyes to avoid rapid strike on to the spandex from residual scour alkali.
- Improved levelling and migration of the cationic dyes on spandex can be achieved by the simultaneous addition to the dyebath of 0.1% Tinegal MR (Huntsman). This product can foam more easily and so additional application 0.5ml/per litre Aphrogene NS (non silicone anti-foam from Uniqema) can be helpful.
- Glaubers salt retards cationic dyes on spandex also improves levelling.
- Non-ionic anti-precipitants Uniperol KA (BASF) at 0.25% level can reduce precipitation risks in single bath dyeing applications. Amphoteric -Albegal A (Huntsman) can be used where foaming is a problem.

## Claims

1. An article comprising a fabric wherein said fabric comprises:
(a) a cationic dyeable polyurethane elastic yarn dyed by a cationic dye, and
(b) an acid dyeable yarn selected from the group consisting of polyamide, proteinaceous, and combinations thereof, dyed by an acid dye;
wherein the fabric has a uniform color, wherein uniform color means that the color of the fabric as measured by a-color, b-color, and L-value in CIELAB L*a*b* color space is within 10% of the values that are obtained by removing the cationic dyeable polyurethane elastic yarn from the fabric;
and wherein the fabric comprises from greater than 0 up to 60% by weight of the cationic dyeable polyurethane elastic yarn.

2. The article of claim 1, wherein said fabric includes a construction selected from circular knit, warp knit, and woven.

3. The article of claim 1, wherein said acid dyeable yarn is selected from the group consisting of polyamide, silk, wool, mohair, angora, alpaca and combinations thereof.

4. The article of claim 3, wherein said acid dyeable yarn is selected from the group consisting of mohair, angora, alpaca and combinations thereof.

5. A method for preparing a fabric comprising:
(a) providing a fabric comprising:
(i) a cationic dyeable polyurethane elastic yarn, and
(ii) an acid dyeable yarn selected from the group consisting of polyamide, proteinaceous, and combinations thereof;
(b) contacting said fabric with a cationic dye, and
(c) contacting said fabric with an acid dye;
wherein said fabric has uniform color, wherein uniform color means that the color of the fabric as measured by a-color, b-color, and L-value in CIELAB L*a*b* color space is within 10% of the values that are obtained by removing the cationic dyeable polyurethane elastic yarn from the fabric;
and wherein the fabric comprises from greater than 0 up to 60% by weight of the cationic dyeable polyurethane elastic yarn.

6. The method of claim 5, wherein said acid dyeable yarn is selected from the group consisting of mohair, angora, alpaca and combinations thereof.

7. The article of claim 1 or the method of claim 5, wherein the acid dye is selected from the group consisting of Acid Yellows 24, 40, 59, 159, 184, 204 and 246, Acid Oranges 142 and 156, Acid Reds 50, 51, 52, 138, 151, 299, 361, 362, Acid Greens 104 and 108, Acid Blues 113, 171, 185, 193, 277 and 324, Acid Violet 90, Acid Brown 298, Acid Blacks 52, 131:1, 132:1, 172, 187 and 194, Lanaset Blue 2R, Lanaset Navy R, Lanaset Red G, Lanaset Red 2GA, Lanaset Violet B, Lanaset Brown B, Burconyl Brick Red AF-3b, Burconyl Rubine AF-GR, Burconyl Orange AF-3R, Burconyl Green AF-B, Burconyl Brilliant Blue AF-R, Burconyl Royal Blue AF-R, Burconyl Brilliant Yellow AF-4G, Erionyl Red A-3G, Erionyl Blue RL 200, and Nylanthrene Brilliant Blue 2RFF.

8. The article of claim 7 or the method of claim 7, wherein the acid dye is selected from the group consisting of Acid Yellows 24, 40, 59, 159, 184, 204 and 246, Acid Oranges 142 and 156, Acid Reds 50, 51, 52, 138, 151, 299, 361, 362, Acid Greens 104 and 108, Acid Blues 113, 171, 185, 193, 277 and 324, Acid Violet 90, Acid Brown 298, Acid Blacks 52, 131:1, 132:1, 172, 187 and 194.

9. The article of claim 7 or the method of claim 7, wherein the acid dye is selected from the group consisting of Lanaset Blue 2R, Lanaset Navy R, Lanaset Red G, Lanaset Red 2GA, Lanaset Violet B, Lanaset Brown B, Burconyl Brick Red AF-3b, Burconyl Rubine AF-GR, Burconyl Orange AF-3R, Burconyl Green AF-B, Burconyl Brilliant Blue AF-R, Burconyl Royal Blue AF-R, Burconyl Brilliant Yellow AF-4G, Erionyl Red A-3G, Erionyl Blue RL 200, and Nylanthrene Brilliant Blue 2RFF.

## Patentansprüche

1. Gegenstand, umfassend ein Gewebe, wobei das Gewebe Folgendes umfasst:
(a) ein kationisch färbbares elastisches Polyurethangarn, das mit einem kationischen Farbstoff gefärbt ist, und
(b) ein mit Säure färbbares Garn, ausgewählt aus der Gruppe bestehend aus Polyamid, proteinös, und Kombinationen davon, gefärbt mit einem sauren Farbstoff;
wobei das Gewebe eine einheitliche Farbe aufweist, wobei einheitliche Farbe bedeutet, dass die Farbe des Gewebes, gemessen anhand der a-Farbe, der b-Farbe und des L-Werts im CIELAB L*a*b-Farbraum, innerhalb von 10 % der Werte liegt, die erhalten werden, indem das kationisch färbbare elastische Polyurethangarn aus dem Gewebe entfernt wird;
und wobei das Gewebe mehr als 0 bis 60 Gew.-% des kationisch färbbaren elastischen Polyurethangarns umfasst.

2. Gegenstand nach Anspruch 1, wobei das Gewebe eine Konstruktion umfasst, die ausgewählt ist aus Rundgewirke, Kettengewirke und Fasergewebe.

3. Gegenstand nach Anspruch 1, wobei das mit Säure färbbare Garn aus der Gruppe ausgewählt ist, die aus Polyamid, Seide, Wolle, Mohair, Angora, Alpaka und Kombinationen davon besteht.

4. Gegenstand nach Anspruch 3, wobei das mit Säure färbbare Garn aus der Gruppe bestehend aus Mohair, Angora, Alpaka und Kombinationen davon ausgewählt ist.

5. Verfahren zum Herstellen eines Gewebes, umfassend:
(a) Bereitstellen eines Gewebes, umfassend:
(i) ein kationisch färbbares elastisches Polyurethangarn und
(ii) ein mit Säure färbbares Garn, ausgewählt aus der Gruppe bestehend aus Polyamid, proteinös, und Kombinationen davon;
(b) Kontaktieren des Gewebes mit einem kationischen Farbstoff und
(c) Kontaktieren des Gewebes mit einem sauren Farbstoff;
wobei das Gewebe eine einheitliche Farbe aufweist, wobei einheitliche Farbe bedeutet, dass die Farbe des Gewebes, gemessen anhand der a-Farbe, der b-Farbe und des L-Werts im CIELAB L*a*b-Farbraum, innerhalb von 10 % der Werte liegt, die erhalten werden, indem das kationische färbbare elastische Polyurethangarn aus dem Gewebe entfernt wird;
und wobei das Gewebe mehr als 0 bis 60 Gew.-% des kationisch färbbaren elastischen Polyurethangarns umfasst.

6. Verfahren nach Anspruch 5, wobei das mit Säure färbbare Garn aus der Gruppe bestehend aus Mohair, Angora, Alpaka und Kombinationen davon ausgewählt ist.

7. Gegenstand nach Anspruch 1 oder Verfahren nach Anspruch 5, wobei der saure Farbstoff aus der Gruppe bestehend aus den sauren Gelb-Farbstoffen 24, 40, 59, 159, 184, 204 und 246, den sauren Orange-Farbstoffen 142 und 156, den sauren Rot-Farbstoffen 50, 51, 52, 138, 151, 299, 361, 362, den sauren Grün-Farbstoffen 104 und 108, den sauren Blau-Farbstoffen 113, 171, 185, 193, 277 und 324, dem sauren Violett-Farbstoff 90, dem sauren Braun-Farbstoff 298, den sauren Schwarz-Farbstoffen 52, 131:1, 132:1, 172, 187 und 194, Lanaset Blau 2R, Lanaset Navy R, Lanaset Rot G, Lanaset Rot 2GA, Lanaset Violett B, Lanaset Braun B, Burconyl Ziegelrot AF-3b, Burconyl Rubin AF-GR, Burconyl Orange AF-3R, Burconyl Grün AF-B, Burconyl Brilliantblau AF-R, Burconyl Royalblau AF-R, Burconyl Brilliantgelb AF-4G, Erionyl Rot A-3G, Erionyl Blau RL 200 und Nylanthren Brillantblau 2RFF ausgewählt ist.

8. Gegenstand nach Anspruch 7 oder Verfahren nach Anspruch 7, wobei der saure Farbstoff aus der Gruppe bestehend aus den sauren Gelb-Farbstoffen 24, 40, 59, 159, 184, 204 und 246, den sauren Orange-Farbstoffen 142 und 156, den sauren Rot-Farbstoffen 50, 51, 52, 138, 151, 299, 361, 362, den sauren Grün-Farbstoffen 104 und 108, den sauren Blau-Farbstoffen 113, 171, 185, 193, 277 und 324, dem sauren Violett-Farbstoff 90, dem sauren Braun-Farbstoff 298, den sauren Schwarz-Farbstoffen 52, 131:1, 132:1, 172, 187 und 194 ausgewählt ist.

9. Gegenstand nach Anspruch 7 oder Verfahren nach Anspruch 7, wobei der saure Farbstoff aus der Gruppe bestehend aus Lanaset Blau 2R, Lanaset Navy R, Lanaset Rot G, Lanaset Rot 2GA, Lanaset Violett B, Lanaset Braun B, Burconyl Ziegelrot AF-3b, Burconyl Rubin AF-GR, Burconyl Orange AF-3R, Burconyl Grün AF-B, Burconyl Brilliantblau AF-R, Burconyl Royalblau AF-R, Burconyl Brilliantgelb AF-4G, Erionyl Rot A-3G, Erionyl Blau RL 200 und Nylanthren Brillantblau 2RFF ausgewählt ist.

## Revendications

1. Article comprenant un tissu, dans lequel ledit tissu comprend :
(a) un fil élastique de polyuréthane capable d'être teint par teinture cationique teint par un colorant cationique, et
(b) un fil capable d'être teint par teinture acide sélectionné dans le groupe constitué de polyamide, protéique et de combinaisons de ceux-ci, teint par un colorant acide ;
dans lequel le tissu a une couleur uniforme, une couleur uniforme signifiant que la couleur du tissu mesurée par une couleur a, une couleur b, et une valeur L dans l'espace colorimétrique CIELAB L*a*b* ne s'écarte pas de plus de 10 % des valeurs obtenues en retirant le fil élastique de polyuréthane capable d'être teint par teinture cationique du tissu ;
et dans lequel le tissu comprend de plus de 0 à 60 % en poids du fil élastique de polyuréthane capable d'être teint par teinture cationique.

2. Article selon la revendication 1, dans lequel ledit tissu comprend une construction sélectionnée parmi un tricot circulaire, un tricot chaîne à base jersey, et un tissu tissé.

3. Article selon la revendication 1, dans lequel ledit fil capable d'être teint par teinture acide est sélectionné dans le groupe constitué du polyamide, de la soie, de la laine, du mohair, de l'angora, de l'alpaga, et de combinaisons de ceux-ci.

4. Article selon la revendication 3, dans lequel ledit fil capable d'être teint par teinture acide est sélectionné dans le groupe constitué du mohair, de l'angora, de l'alpaga, et de combinaisons de ceux-ci.

5. Procédé de préparation d'un tissu comprenant :
(a) la fourniture d'un tissu comprenant :
(i) un fil élastique de polyuréthane capable d'être teint par teinture cationique, et
(ii) un fil capable d'être teint par teinture acide sélectionné dans le groupe constitué de fils de polyamide, de fils constitués de matériaux protéiques, et de combinaisons de ceux-ci ;
(b) la mise en contact dudit tissu avec un colorant cationique, et
(c) la mise en contact dudit tissu avec un colorant acide ;
dans lequel ledit tissu a une couleur uniforme, une couleur uniforme signifiant que la couleur du tissu mesurée par une couleur a, une couleur b, et une valeur L dans l'espace colorimétrique CIELAB L*a*b* ne s'écarte pas de plus de 10 % des valeurs obtenues en retirant le fil élastique de polyuréthane capable d'être teint par teinture cationique du tissu ;
et dans lequel le tissu comprend de plus de 0 à 60 % en poids du fil élastique de polyuréthane capable d'être teint par teinture cationique.

6. Procédé selon la revendication 5, dans lequel ledit fil capable d'être teint par teinture acide est sélectionné dans le groupe constitué du mohair, de l'angora, de l'alpaga, et de combinaisons de ceux-ci.

7. Article selon la revendication 1 ou procédé selon la revendication 5, dans lequel le colorant acide est sélectionné dans le groupe constitué des jaunes acides 24, 40, 59, 159, 184, 204 et 246, des oranges acides 142 et 156, des rouges acides 50, 51, 52, 138, 151, 299, 361, 362, des verts acides 104 et 108, des bleus acides 113, 171, 185, 193, 277 et 324, du violet acide 90, du brun acide 298, des noirs acides 52, 131:1, 132:1, 172, 187 et 194, du bleu Lanaset 2R, du bleu marine Lanaset R, du rouge Lanaset G, du rouge Lanaset 2GA, du violet Lanaset B, du brun Lanaset B, du rouge brique Burconyl AF-3b, du rubis Burconyl AF-GR, de l'orange Burconyl AF-3R, du vert Burconyl AF-B, du bleu brilliant Burconyl AF-R, du bleu roi Burconyl AF-R, du jaune brillant Burconyl AF-4G, du rouge Erionyl A-3G, du bleu Erionyl RL 200, et du bleu brillant Nylanthrene 2RFF.

8. Article selon la revendication 7 ou procédé selon la revendication 7, dans lequel le colorant acide est sélectionné dans le groupe constitué des jaunes acides 24, 40, 59, 159, 184, 204 et 246, des oranges acides 142 et 156, des rouges acides 50, 51, 52, 138, 151, 299, 361, 362, des verts acides 104 et 108, des bleus acides 113, 171, 185, 193, 277 et 324, du violet acide 90, du brun acide 298, des noirs acides 52, 131:1, 132:1, 172, 187 et 194.

9. Article selon la revendication 7 ou procédé selon la revendication 7, dans lequel le colorant acide est sélectionné dans le groupe constitué du bleu Lanaset 2R, du bleu marine Lanaset R, du rouge Lanaset G, du rouge Lanaset 2GA, du violet Lanaset B, du brun Lanaset B, du rouge brique Burconyl AF-3b, du rubis Burconyl AF-GR, de l'orange Burconyl AF-3R, du vert Burconyl AF-B, du bleu brilliant Burconyl AF-R, du bleu roi Burconyl AF-R, du jaune brillant Burconyl AF-4G, du rouge Erionyl A-3G, du bleu Erionyl RL 200, et du bleu brillant Nylanthrene 2RFF.
